

## 1

2,979,406

## SINGLE POWDER PHOTOGRAPHIC DEVELOPERS

John B. Taylor and Jerry S. Krizka, Binghamton, N.Y., assignors to General Aniline & Film Corporation, New York, N.Y., a corporation of Delaware

No Drawing. Filed Apr. 11, 1956, Ser. No. 577,452

8 Claims. (Cl. 96—66)

The present invention relates to single powder photographic developers in which all of the essential ingredients of the developer are intimately admixed in dry powder form and, more particularly, to an improved stabilizer for such developers.

Single powder photographic developers contain as their essential ingredients one or more organic developing agents such as N-methyl-p-aminophenol, hydroquinone, 1-phenyl-3-pyrazolidone, para-aminophenol monohydrochloride, pyrogallol, an alkali such as sodium carbonate, borax, sodium metaborate or the like, a preservative such as an alkali metal sulfite and an anti-fogging agent such as potassium bromide. Under ordinary conditions of mixing and storage, such dry developers undergo decomposition reactions which adversely affect the photographic activity of the developers.

The art has been cognizant of this phenomenon and, in an effort to avoid it, has provided for the presence in such developers of an acidic stabilizer such as phthalic acid, anhydrous oxalic acid, boric anhydride, metaboric acid, potassium metabisulfite and the like. While these various acid stabilizers serve to promote the keeping qualities of such developers, they do not lead to optimum results, as is evident by the fact that developers containing the same generally discolor within a period of two to three months.

It is known that alkali metal polyphosphates have utility in photographic developers as sequestering agents for the salts which cause hardness of water. When used for this purpose, the alkali metal phosphates are employed in small amounts, i.e., usually less than one gram per liter.

We have now discovered that the stabilizing ability of the usual acidic stabilizers for single powder photographic developers is surprisingly promoted by using with said stabilizers, a substantially higher quantity of an alkali metal polyphosphate than is used when the polyphosphate is to operate as a sequestering agent. Dry powder developers containing the usual acidic stabilizers with such higher quantities of alkali metal polyphosphates constitute the purposes and objects of the present invention.

The developers which are contemplated herein contain as their essential components an alkali metal polyphosphate, an organic developing agent, an alkali, a preservative, an anti-fogging agent and an acid stabilizer. Developers with these components which we have found to be stable during mixing and during storage for considerable periods of time may be compounded in the following proportions, it being understood that the resulting dry powder is to be used to make a liter of developing solution:

|                               |       |           |
|-------------------------------|-------|-----------|
| An alkali metal polyphosphate | Grams | 1 to 8    |
| Organic developing agent      |       | 4 to 15   |
| Alkali                        |       | 5 to 100  |
| Preservative                  |       | 30 to 120 |
| Anti-fogging agent            |       | .5 to 2   |
| Acid stabilizer               |       | .5 to 12  |

## 2

Any of the usual alkali metal polyphosphates may be employed such as sodium hexametaphosphate, potassium hexametaphosphate and the like. Best results, however, are achieved by use of the sodium hexametaphosphate and the use of this compound is, accordingly, preferred.

The photographic developing agent may be any of those previously mentioned and it may be used alone or in admixture with other developing agents. Typically, we may use a mixture of N-methyl-p-aminophenol and hydroquinone, metol and 1-phenyl-3-pyrazolidone (phenidone), phenidone and hydroquinone or phenidone, N-methyl-p-aminophenol and hydroquinone.

The preservative is preferably sodium sulfite usually in the anhydrous condition and the anti-fogging agent is potassium bromide. The alkali may be any of those used in compounding photographic developers, such as sodium carbonate, sodium hydroxide, sodium tetraborate, sodium metaborate or the like.

In compounding the aforesaid developer mixtures, one may proceed by first mixing the alkali metal polyphosphate with the acidic stabilizer or stabilizers, adding and admixing the alkali, then the developing agent and finally the other ingredients. However, if it be preferred, all the ingredients may be admixed simultaneously.

It is to be emphasized that the alkali metal polyphosphates, per se, have no stabilizing effect whatsoever on single powder photographic developers. In other words, no useful result would be performed by admixing an alkali metal phosphate such as sodium hexametaphosphate with the essential components of a single powder photographic developer from the standpoint of achieving stability thereof, either in the preparation or in storage of such developer. However, when the alkali metal polyphosphate is present with one of the usual acidic stabilizers, it serves to greatly promote the stabilizing effect, an action which appears to be synergistic in character. Thus, as noted, single powder developers containing sodium hexametaphosphate even in the quantities heretofore specified, in the absence of an acidic stabilizer, show no improvement over similar single powder developers free from the acidic stabilizer. Single powder developers containing the usual acidic stabilizers absent the sodium hexametaphosphate discolor in a period of a few months. When, however, the acidic stabilizers and the alkali metal polyphosphate in the noted quantity are present together in a single powder developer, the stability of the developer is greatly magnified and no discoloration appears even after storing the developer for more than 12 months. It is manifest, the facts being as stated, that the results must be attributable to some peculiar coaction between the hexametaphosphate and the acidic stabilizer which serves to greatly intensify the stabilizing action of the acidic component.

The following examples will serve to illustrate our invention, the parts being by weight.

|                                    | Example I | Grams |
|------------------------------------|-----------|-------|
| Sodium hexametaphosphate           |           | 2.0   |
| Ethylene diamine tetra acetic acid |           | 0.7   |
| Phthalic acid                      |           | 0.5   |
| 65 Potassium metabisulfite         |           | 6.0   |
| Sodium carbonate, monohydrate      |           | 30.0  |
| Sodium sulfite, anhydrous          |           | 40.0  |
| N - methyl-p-aminophenol           |           | 2.0   |
| 70 Hydroquinone                    |           | 5.0   |
| Potassium bromide                  |           | 1.0   |

## Example II

|                                    | Grams |
|------------------------------------|-------|
| Sodium hexametaphosphate           | 3.0   |
| Ethylene diamine tetra acetic acid | 1.0   |
| Oxalic acid (anhydrous)            | 0.3   |
| Potassium metabisulfite            | 2.5   |
| Borax, pentahydrate                | 5.0   |
| Sodium sulfite, anhydrous          | 100.0 |
| N - methyl-p-aminophenol           | 1.2   |
| Hydroquinone                       | 8.0   |
| Potassium bromide                  | 0.5   |

## Example III

|                                    | Grams |
|------------------------------------|-------|
| Sodium hexametaphosphate           | 4.0   |
| Ethylene diamine tetra acetic acid | 0.8   |
| Phthalic acid                      | 1.0   |
| Potassium metabisulfite            | 10.0  |
| Sodium carbonate, monohydrate      | 80.0  |
| Sodium sulfite, anhydrous          | 50.0  |
| Phenidone                          | .25   |
| N - methyl-p-aminophenol           | 1.0   |
| Hydroquinone                       | 7.5   |
| Potassium bromide                  | 1.5   |

## Example IV

|                                    | Grams |
|------------------------------------|-------|
| Sodium hexametaphosphate           | 6.0   |
| Ethylene diamine tetra acetic acid | 0.8   |
| Metaboric acid                     | 2.0   |
| Potassium metabisulfite            | 3.0   |
| Sodium carbonate, monohydrate      | 8.0   |
| Sodium sulfite, anhydrous          | 100.0 |
| Phenidone                          | .15   |
| Hydroquinone                       | 4.5   |
| Potassium Bromide                  | 0.5   |

## Example V

|                                    | Grams |
|------------------------------------|-------|
| Sodium hexametaphosphate           | 2.0   |
| Ethylene diamine tetra acetic acid | 0.8   |
| Boric anhydride                    | 0.75  |
| Potassium metabisulfite            | 6.0   |
| Sodium carbonate, monohydrate      | 20.0  |
| Sodium sesqui-carbonate            | 8.0   |
| Sodium sulfite, anhydrous          | 50.0  |
| N - methyl-p-aminophenol           | 3.5   |
| Hydroquinone                       | 7.0   |
| Potassium bromide                  | 1.2   |

The quantity of the developer represented by the above formulae is to be dissolved in water to make one liter of developing solution.

Modifications of the invention will occur to persons skilled in the art. We, therefore, do not intend to be limited in the patent granted except as necessitated by the appended claims.

We claim:

1. A single powder photographic developing composition containing an organic photographic developing agent, an alkali metal sulfite, an alkali selected from the group consisting of sodium carbonate, sodium hydroxide, sodium tetraborate and sodium metaborate, an anti-fogging agent, a sufficient amount of an acid stabilizer selected from the group consisting of phthalic acid, anhydrous oxalic acid, boric anhydride, metaboric acid and potassium metabisulfite to produce 0.5 to 12 grams per liter in solution and a sufficient amount of alkali metal hexametaphosphate to produce at least 1 gram per liter in solution.

2. A single powder developing composition containing sufficient of the following ingredients to produce, upon dissolution, a developing solution having the fol-

lowing amounts of these ingredients per liter of solution:

|                                                                                                                                                         | Grams     |
|---------------------------------------------------------------------------------------------------------------------------------------------------------|-----------|
| 5 Alkali metal hexametaphosphate                                                                                                                        | 1 to 8    |
| Organic photographic developing agent                                                                                                                   | 4 to 15   |
| An alkali selected from the group consisting of sodium carbonate, sodium hydroxide, sodium tetraborate and sodium metaborate                            | 5 to 100  |
| 10 Alkali metal bisulfite                                                                                                                               | 30 to 120 |
| Antifogging agent                                                                                                                                       | .5 to 2   |
| Acid stabilizer selected from the group consisting of phthalic acid, anhydrous oxalic acid, boric anhydride, metaboric acid and potassium metabisulfite | .5 to 12  |

3. The composition as defined in claim 1 wherein sufficient alkali metal hexametaphosphate is employed to produce about 1 to 8 grams thereof per liter of developer solution.

4. A single powder developing composition containing sufficient of the following ingredients to produce, upon dissolution, a developing solution having the following amounts of these ingredients per liter of solution:

|                                    | Grams |
|------------------------------------|-------|
| Sodium hexametaphosphate           | 2     |
| Ethylene diamine tetra acetic acid | .7    |
| Phthalic acid                      | .5    |
| 30 Potassium metabisulfite         | 6     |
| Sodium carbonate, monohydrate      | 30    |
| Sodium sulfite, anhydrous          | 40    |
| N - methyl-p-aminophenol           | 2     |
| 35 Hydroquinone                    | 5     |
| Potassium bromide                  | 1     |

5. A single powder developing composition containing sufficient of the following ingredients to produce, upon dissolution, a developing solution having the following amounts of these ingredients per liter of solution:

|                                    | Grams |
|------------------------------------|-------|
| 45 Sodium hexametaphosphate        | 3     |
| Ethylene diamine tetra acetic acid | 1     |
| Oxalic acid (anhydrous)            | .3    |
| Potassium metabisulfite            | 2.5   |
| Borax, pentahydrate                | 5     |
| 50 Sodium sulfite, anhydrous       | 100   |
| N - methyl-p-aminophenol           | 1.2   |
| Hydroquinone                       | 8     |
| Potassium bromide                  | .5    |

55 6. A single powder developing composition containing sufficient of the following ingredients to produce, upon dissolution, a developing solution having the following amounts of these ingredients per liter of solution:

|                                    | Grams |
|------------------------------------|-------|
| 60 Sodium hexametaphosphate        | 4     |
| Ethylene diamine tetra acetic acid | .8    |
| Phthalic acid                      | 1     |
| 65 Potassium metabisulfite         | 10    |
| Sodium carbonate, monohydrate      | 80    |
| Sodium sulfite, anhydrous          | 50    |
| Phenidone                          | .25   |
| N - methyl-p-aminophenol           | 1     |
| 70 Hydroquinone                    | 7.5   |
| Potassium bromide                  | 1.5   |

7. A single powder developing composition containing sufficient of the following ingredients to produce, upon dissolution, a developing solution having the fol-

lowing amounts of these ingredients per liter of solution:

|                                    | Grams | Grams |
|------------------------------------|-------|-------|
| Sodium hexametaphosphate           | 6     | 5     |
| Ethylene diamine tetra acetic acid | .8    |       |
| Metaboric acid                     | 2     |       |
| Potassium metabisulfite            | 3     |       |
| Sodium carbonate, monohydrate      | 8     |       |
| Sodium sulfite, anhydrous          | 100   | 10    |
| Phenidone                          | .15   |       |
| Hydroquinone                       | 4.5   |       |
| Potassium bromide                  | .5    |       |

8. A single powder developing composition containing sufficient of the following ingredients to produce, upon dissolution, a developing solution having the following amounts of these ingredients per liter of solution:

|                                    | Grams | Grams |
|------------------------------------|-------|-------|
| Sodium hexametaphosphate           | 2     | 20    |
| Ethylene diamine tetra acetic acid | .8    |       |
| Boric anhydride                    | .75   |       |
| Potassium metabisulfite            | 6     |       |
| Sodium carbonate, monohydrate      | 20    |       |

|                           | Grams |
|---------------------------|-------|
| Sodium sesqui-carbonate   | 8     |
| Sodium sulfite, anhydrous | 50    |
| N - methyl-p-aminophenol  | 3.5   |
| Hydroquinone              | 7     |
| Potassium bromide         | 1.2   |

#### References Cited in the file of this patent

##### UNITED STATES PATENTS

|           |              |               |
|-----------|--------------|---------------|
| 2,239,284 | Draisbach    | Apr. 22, 1941 |
| 2,541,470 | Henn et al.  | Feb. 13, 1951 |
| 2,610,122 | John et al.  | Sept. 9, 1952 |
| 2,688,549 | James et al. | Sept. 7, 1954 |

##### FOREIGN PATENTS

|         |               |               |
|---------|---------------|---------------|
| 520,753 | Great Britain | May 2, 1940   |
| 734,534 | Germany       | Nov. 4, 1943  |
| 743,534 | Germany       | Dec. 29, 1943 |

##### OTHER REFERENCES

Photo-Lab-Index, pages 13-35 and pages 13-36, Morgan and Lester Publishers, New York, N.Y.

UNITED STATES PATENT OFFICE  
CERTIFICATE OF CORRECTION

Patent No. 2,979,406

April 11, 1961

John B. Taylor et al.

It is hereby certified that error appears in the above numbered patent requiring correction and that the said Letters Patent should read as corrected below.

Column 2, line 10, for "metol" read -- N-methyl-p-aminophenol --.

Signed and sealed this 10th day of October 1961.

(SEAL)

Attest:

ERNEST W. SWIDER

Attesting Officer

DAVID L. LADD

Commissioner of Patents  
USCOMM-DC